

## UNITED STATES PATENT OFFICE

2,652,363

## GREASE COMPOSITIONS

Harold A. Woods and Loren C. Bollinger, Martinez, Calif., assignors to Shell Development Company, Emeryville, Calif., a corporation of Delaware

No Drawing. Application December 29, 1951,  
Serial No. 264,231

11 Claims. (Cl. 252—34.7)

1

This invention relates to special grease compositions. More particularly it is concerned with greases resistant to the solvent action of water and of light hydrocarbons such as gasoline.

In the lubrication of metal connections for pipe lines and flexible metallic hoses and the like, difficulties are encountered when the fluid carried by the pipe line dissolves the lubricant away from the connections. This becomes a matter of great concern in military applications and especially for such purposes as fuel transfer between planes during flight. Greases comprising ordinary metallic soaps and mineral lubricating oils are much too gasoline sensitive to be used for such purposes. On the other hand, it is undesirable to have a grease which is entirely insoluble in gasoline or water since between periods of use the grease forms hard metallic residues which plug the connections and cause other difficulties of operation. A number of greases have been proposed for use on apparatus such as valve connections and the like wherein the grease is composed substantially entirely of gasoline-resistant ingredients. Hence, the art has proposed the use of greases which are known to be too sensitive to the action of gasoline for critical uses such as in-flight transmission of fuel and, on the other hand, has proposed lubricants which are substantially insoluble in both water and gasoline.

It is an object of the present invention to provide greases which are resistant to washing away by the action of gasoline or water but which are not entirely insoluble therein. It is another object of this invention to provide greases for temporary use and which do not cause the formation of hard metallic residues. Other objects will become apparent during the following discussion.

Now, in accordance with the present invention, it has been found that gasoline and water resistant greases may be formed by utilizing as the major liquid components a mixture of a water soluble polyoxyalkylene fluid and a partial ester of a polyhydric alcohol having less than six carbon atoms with a higher fatty acid. Additionally, it has been determined that other advantages are gained by the presence of a combination of an aromatic amine and a substituted oxazoline, all as more particularly described hereinafter. More specifically a grease having optimum properties comprises a gelling amount of an amine soap of a higher fatty acid. The latter type of soap is preferably dispersed in a partial ester of a higher hydroxy fatty acid mixed with a water soluble polyoxyalkylene compound. The chief

2

advantages gained by the use of this type of composition comprise the essentially gasoline and water resistant character of the entire composition while, at the same time, the amine soap leaves a soft residue which tends to be flushed away to a large extent during use in the transmission of gasoline, or other light hydrocarbon, thus leaving a film on the connecting parts of the mixture of gasoline resistant lubricants, namely, the partial ester and the polyoxyalkylene fluid. Hence, this type of composition comprises an advance over the two types of greases already proposed, namely, those which are sensitive in both the fluid and gelling components to the solvent action of gasoline and the opposite type of composition which is entirely insoluble in light hydrocarbons and water.

*The soaps*

20 The soaps with which the present invention is concerned comprise particularly the hydroxyalkylamine soaps of higher fatty acids. Preferably, these fatty acids have at least 12 carbon atoms and optimum results are obtained when the fatty acid has between 16 and 20 carbon atoms. While satisfactory results may be obtained with ordinary saturated fatty acids, the best solubility relationships are gained by the use of unsaturated fatty acids and, more especially, by employing unsaturated hydroxy fatty acids. 25 Suitable materials include the following: capric acid, undecylic acid, lauric acid, myristic acid, stearic acid, oleic acid, 9-, 10-, 11-, 12-, or 13-hydroxy stearic acids, 10-, or 15-hydroxy palmitic acids, 10-hydroxy myristic acid, 5,6-dihydroxy 30 stearic acid, 2,11-dihydroxy palmitic acid, 12-hydroxy oleic (ricinoleic) acid, 12-hydroxy-9,10-hexadecenoic (palmitoleic) acid, and 12-hydroxy-9,10-tetradecenoic (myristoleic) acid.

The above types of fatty acids are to be reacted 35 to form soaps with alkanolamines having less than six carbon atoms per alkanol radical and, preferably, with trialkanolamines. The most commonly available species and one which has been found to give satisfactory results is triethanolamine. Other species suitable for the present purpose are exemplified by the following list: mono-ethanolamine, di-ethanolamine, di-amino-isopropanol, di-n-propanolamine, tri-isopropanolamine, butanolamines.

40 It will be apparent from the list of alkanolamines and higher fatty acids given above that the preferred type of soap comprises the soap of a trialkanolamine with an unsaturated hydroxy fatty acid having more than twelve carbon atoms in the molecule. However, derivatives of certain

natural products may be employed as well. For example, the triethylene amine soap of hydrogenated castor oil acids is suitable in addition to the following typical soaps:

Triethanolamine ricinoleate  
 Diethanolamine ricinoleate  
 Tri-isopropanolamine ricinoleate  
 Mono-butanolamine ricinoleate  
 Triethanolamine-12-hydroxystearate  
 Triethanolamine-10-hydroxy myristate  
 Triethanolamine-9,10-dihydroxy palmitate  
 Triethanolamine-12-hydroxy palmitoleate

### *The partial esters*

The fluid components of the present gasoline resistant greases comprise two essential types. The first of these is a partial ester of a poly-hydroxy alcohol, said alcohol having from two to ten carbon atoms with higher fatty acids. Optimum results are obtained by the use of poly-hydric alcohols having from two to five carbon atoms and, preferably, are glycol or glyceryl partial esters of unsaturated fatty acids, the latter having at least twelve carbon atoms per molecule. More especially, excellent gasoline-resistant properties are obtained by the use of partial glyceryl esters of unsaturated hydroxy fatty acids. The list which follows presents typical partial esters suitable for use in the present greases:

Glyceryl monoricinoleate  
Glycol monoricinoleate  
Pentaerythritol monoricinoleate  
Glyceryl diricinoleate  
Carbitol ricinoleate (monoricinoleate of diethyl-  
ene glycol monoethyl ether)  
Glyceryl oleate  
Glycol palmitate  
Glyceryl-mono(12-hydroxystearate)  
Glyceryl-mono(9,10-dihydroxypalmitate)  
Glyceryl-mono(12-hydroxypalmitate)

It will be noted that the above types of partial esters comprise not only the simple partial esters of polyhydric alcohols with higher fatty acids but also comprise the partial esters of high fatty acids with mono-ethers of polyhydric alcohols. These are exemplified by the "Carbitol" ricinoleate. The Carbitol is understood to be diethylene glycol monoethyl ether. Other ethers suitable for this purpose include diethylene glycol monobutyl ether, diethylene glycol monoethylene ether and the mono-ethers of alkylene glycols such as ethylene glycol monobutyl ether.

### *The polyotalkulene fluids*

The third essential component of the present gasoline resistant grease compositions comprises water soluble polyoxyalkylene fluids. It is desirable, of course, to have this fluid not only be soluble in water but also miscible with the partial esters discussed hereinbefore. Preferably they should have a volatility comparable to a medium viscosity lubricating oil but the latter property is not as important as its solubility in water and its lack of solubility in gasoline or other light hydrocarbons. The principal function of these fluids comprises the improvement of resistance to washing away, by gasoline or the like, of the partial esters and at the same time the improvement in the low temperature operating characteristics of the grease. It has been found that greases comprising the ester and soaps, such as triethanolamine ricinoleate, operate fairly satisfactorily only at room temperature or slightly below. The

presence of the additional fluid, such as that described hereinafter as "a water soluble Ucon fluid" improves the gasoline resistance of the grease and, moreover, enables it to be used at low temperatures, such as occur at higher altitudes, in the order of  $-65^{\circ}\text{ F.}$ , without becoming unduly stiff. The water soluble fluids are preferably those composed to a large extent of oxyalkylene units wherein the unit contains from two to ten carbon atoms. The best fluid for the present purpose comprises the mono-ethers of oxyalkylene polymers such as the lower monoalkylene ethers of polyalkylene oxides and glycols. In addition to the ethers of polyalkylene oxides or glycols, esters may be employed and the polymers may be either homo-polymers or co-polymers of two or more monomeric oxides or glycols. Among these will be found trimethylene glycol, ethylene glycol, co-polymers of ethylene glycol and propylene glycol, co-polymers of ethylene oxide and 1-propylene oxide and the like.

It has been found that useful and improved polyoxyalkylene products of relatively high average molecular weight, which are essentially mixtures of true monohydroxy alcohols, may be obtained by the addition to a monohydroxy aliphatic alcohol of a mixture of alkylene oxides containing ethylene oxide and 1-propylene oxide in a ratio preferably from about 50:50 to 75:25 ethylene oxide to 1,2-propylene oxide. By this oxide ratio is meant that in the oxide mixture, which may be used in forming such monohydroxy alcohol addition products, the amount of 1,2-propylene oxide in the mixture is from  $\frac{1}{2}$  to an equal amount of ethylene oxide present by weight.

The reaction which takes place between the alcohol and the ethylene oxide and propylene oxide seems to be a simple addition wherein the alkylene oxide molecules undergo conversion to the corresponding oxyalkylene radicals as illustrated for any given molecule by the following general equation:



wherein ROH is an aliphatic monohydroxy alcohol;  $y$  and  $z$  represent the mols of ethylene oxide and 1,2-propylene oxide, respectively;  $n$  is both 2 and 3 in a single molecule, the total number of times  $n$  has a value of 2 being equal to  $y$  and the total number of times  $n$  has a value of 3 being equal to  $z$ ; and  $x$  is the total number of such oxyalkylene groups, being equal to  $y+z$ .

These polymers are preferably mono-ethers of polyoxyalkylene glycols with monohydric aliphatic alcohols having from one to six carbon atoms and preferably from two to five. The molecular weight is preferably between 500 and 1500. A typical example of this series comprises the mixture of monohydroxy oxyalkylene, oxy-1,2-propylene butyl mono-ethers having an average molecular weight of between 500 and 1500 in which the ethylene oxide and 1,2-propylene oxide are combined therein as oxyethylene and oxy-1,2-propylene groups in a ratio of  $\frac{1}{3}$  part of 1,2-propylene oxide for each part by weight of ethylene oxide, the mono-ethers of said mixture containing in a single molecule both the oxyalkylene and oxy-1,2-propylene groups.

The fluids which have been found to be particularly suitable should have viscosities of between about 50 and 2,000 SUS at 100° F. They usually have viscosity indexes which vary about

90 to 150. The pour points of the lower viscosity members, which are preferred, are between about -90 and -40° F. Their flash points, open cup, are between about 250 and 450° F. They have fire points, open cup, between about 275 and 550° F. The preferred varieties are those which have a viscosity between about 50 and 250 SUS at 100° F.

*The greases*

The greases of the present invention comprise 10 the three essential ingredients in the following proportions:

Amine soap: 5-25% by weight

Water soluble polyoxyalkylene fluid: 20-50% by 15 weight

Partial ester: 30-60% by weight

When proportions of this variety are employed a wide variety of greases may be obtained for particular purposes. Using amounts of soaps between 12 and 20%, one may obtain a grease having a medium consistency and which maintains a lubricating quality even at extremely low temperatures such as lower than -40° F. It is preferred that the weight ratio of polyoxyalkylene fluid to the partial ester be between 2:5 and 4:5. The best results are obtained when the polyoxyalkylene fluid comprises 25-40% of the grease and the partial ester comprises between 55 and 35% by weight of the grease. The examples which follow illustrate typical compositions of the present invention:

Example I—

|                             | Percent by weight | 35 |
|-----------------------------|-------------------|----|
| Triethanolamine ricinoleate | 20                |    |
| 50 HB 100 Ucon fluid        | 30                |    |
| Glyceryl monoricinoleate    | 50                |    |

Example II—

|                             | 40 |
|-----------------------------|----|
| Triethanolamine ricinoleate | 15 |
| 50 HB 100 Ucon fluid        | 33 |
| Glycol monoricinoleate      | 52 |

Example III—

|                                 | 45 |
|---------------------------------|----|
| Triethanolamine ricinoleate     | 10 |
| 50 HB 100 Ucon fluid            | 30 |
| Pentaerythritol monoricinoleate | 60 |

Example IV—

|                                   | 50 |
|-----------------------------------|----|
| Triethanolamine ricinoleate       | 25 |
| 50 HB 100 Ucon fluid              | 20 |
| Diethylene glycol monoricinoleate | 55 |

Example V—

|                             | 55 |
|-----------------------------|----|
| Triethanolamine ricinoleate | 20 |
| 50 HB 100 Ucon fluid        | 50 |
| "Carbitol" monoricinoleate  | 30 |

Example VI—

|                             | 60 |
|-----------------------------|----|
| Triethanolamine ricinoleate | 20 |
| 50 HB 100 Ucon fluid        | 35 |
| Glyceryl diricinoleate      | 45 |

Example VII—

|                            | 65 |
|----------------------------|----|
| Diethanolamine ricinoleate | 18 |
| 50 HB 100 Ucon fluid       | 37 |
| Glyceryl monoricinoleate   | 45 |

Example VIII—

|                          | 70 |
|--------------------------|----|
| Ethanolamine ricinoleate | 22 |
| 50 HB 100 Ucon fluid     | 28 |
| Glyceryl monoricinoleate | 50 |

Example IX—

|                                | 75 |
|--------------------------------|----|
| Di-n-propanolamine ricinoleate | 16 |
| 50 HB 100 Ucon fluid           | 30 |
| Glyceryl monoricinoleate       | 54 |

|                                    | Percent by weight |
|------------------------------------|-------------------|
| Triethanolamine-12-hydroxystearate | 12                |
| 50 HB 100 Ucon fluid               | 34                |
| Glyceryl monoricinoleate           | 54                |

|                                        | Percent by weight |
|----------------------------------------|-------------------|
| Triethanolamine-9,10-dihydroxystearate | 20                |
| 50 HB 100 Ucon fluid                   | 30                |
| Glyceryl monoricinoleate               | 50                |

|                                 | Percent by weight |
|---------------------------------|-------------------|
| Triisopropanolamine ricinoleate | 20                |
| 50 HB 55 Ucon fluid             | 30                |
| Glyceryl monoricinoleate        | 50                |

|                             | Percent by weight |
|-----------------------------|-------------------|
| Triethanolamine ricinoleate | 25                |
| 50 HB 660 Ucon fluid        | 20                |
| Glyceryl monoricinoleate    | 55                |

|                                     | Percent by weight |
|-------------------------------------|-------------------|
| Triethanolamine ricinoleate         | 20                |
| Poly(propylene glycol) mol. wt. 250 | 30                |
| Glyceryl monoricinoleate            | 50                |

|                                        | Percent by weight |
|----------------------------------------|-------------------|
| Triethanolamine ricinoleate            | 20                |
| Poly(trimethylene glycol) mol. wt. 300 | 30                |
| Glyceryl monoricinoleate               | 50                |

|                                                                                   | Percent by weight |
|-----------------------------------------------------------------------------------|-------------------|
| Triethanolamine ricinoleate                                                       | 20                |
| 1/2-ester of butyric acid and poly(ethylene glycol-propylene glycol) mol. wt. 325 | 30                |
| Glyceryl monoricinoleate                                                          | 50                |

|                                                                        | Percent by weight |
|------------------------------------------------------------------------|-------------------|
| Triethanolamine ricinoleate                                            | 20                |
| 1/2 butyl ether of poly(ethylene glycol-propylene glycol) mol. wt. 600 | 30                |
| Glyceryl monoricinoleate                                               | 50                |

|                                  | Percent by weight |
|----------------------------------|-------------------|
| Triethanolamine ricinoleate      | 20                |
| 50 HB 100 Ucon fluid             | 30                |
| Glyceryl mono-12-hydroxystearate | 50                |

|                                        | Percent by weight |
|----------------------------------------|-------------------|
| Triethanolamine ricinoleate            | 20                |
| 50 HB 100 Ucon fluid                   | 30                |
| Glyceryl mono-(9,10-dihydroxystearate) | 50                |

|                             | Percent by weight |
|-----------------------------|-------------------|
| Triethanolamine ricinoleate | 19                |
| 50 HB 100 Ucon fluid        | 33                |
| Glyceryl monoricinoleate    | 47.5              |
| Phenyl alpha-naphthylamine  | 0.5               |

|                                                                 | Percent by weight |
|-----------------------------------------------------------------|-------------------|
| Triethanolamine ricinoleate                                     | 18.0              |
| 50 HB 100 Ucon fluid                                            | 32.0              |
| Glyceryl monoricinoleate                                        | 47.0              |
| Phenyl alpha-naphthylamine                                      | 0.5               |
| Oleic acid salt of 2-heptadecyl-hydroxy-methyl-4-ethyloxazoline | 2.5               |

The oxidation and corrosion characteristics of these compositions are improved to an outstanding extent by the inclusion of a combination of an aromatic amine and a higher fatty acid salt of a substituted oxazoline having the general configuration:



wherein R<sub>1</sub> and R<sub>2</sub> are hydrogen, alkyl, hydroxy-alkyl, aryl- or acyl-oxyalkyl radicals, and R<sub>3</sub> and R<sub>4</sub> are either hydrogen or alkyl substituents. Typical members of this group will be found in U. S. Patent 2,402,791. Additives which may be employed include especially those having at least six carbon atoms and preferably twelve or more carbon atoms. They may be saturated or unsaturated acids and, furthermore, may contain hydroxy groups resulting in a hydroxy fatty acid. Typical species meeting these requirements include capric acid, lauric acid, myristic acid, oleic acid, stearic acid, 12-hydroxy oleic acid, 12-hydroxy stearic acid and mixtures of acids from natural glycerides such as fish oil fatty acids, coconut oil fatty acids, and acids from animal fats and oils. Typical oxazolines which may be utilized in salt formation with the above acids include the following: the oxazolines utilized in preparing the products of the present invention may be any of a number of such compounds, as for example, 2-ethyl-4-hydroxymethyl-4-methyloxazoline, 2-isopropyl-4-hydroxymethyl-4-methyloxazoline, 2-heptyl-4-hydroxymethyl-4-ethyloxazoline, 2-tridecyl-4-hydroxymethyl-4-methyloxazoline, 2-octyl-4-hydroxymethyl-4-ethyloxazoline, 2-hendecyl-4-hydroxymethyl-4-methyloxazoline, 2-hendecyl-4-hydroxymethyl-4-ethyloxazoline, 2-heptyl-4,4-bis(hydroxymethyl)oxazoline, 2-octyloxazoline, 2-hendecyl-4,4-bis(hydroxymethyl)oxazoline, 2-hendecyloxazoline, 2-hendecyl-4,4-dimethyloxazoline, and the like.

Suitable salts of the above class include the oleic acid salt of 2-heptyl-4-hydroxymethyl-4-ethyloxazoline; the 12-hydroxystearic acid salt of 2-ethyl-4-hydroxymethyl-4-methyloxazoline and the stearic acid salt of 2-decyl-4,4-dimethyloxazoline.

The aromatic amines to be combined with these oxazoline salts include, particularly, polycycloamines of which the preferred species is phenyl-alpha-naphthylamine. It is preferred that the group contain at least one phenyl radical and that in addition thereto another hydrocarbon group or substituted hydrocarbon group be directly attached to the nitrogen atom. These amino compounds therefore comprise materials having the structural configuration:



wherein R is a hydrocarbon or a substituted hydrocarbon radical. Typical species include phenyl-beta-naphthylamine, diphenylamine, phenylstearylamine and the like.

We claim as our invention:

1. A gasoline-resistant grease comprising a gelling amount of hydroxyalkylamine soap of a higher fatty acid, 20-50% by weight of a water soluble polyoxalkylene fluid and 30-60% by weight of a partial ester of a polyhydric alcohol having less than six carbon atoms with a higher fatty acid.

2. A gasoline-resistant grease comprising a gelling amount of triethanolamine ricinoleate, 20-50% by weight of a water soluble monohydroxy oxyethylene oxy-1,2-propylene butyl mono-ether having an average molecular weight of at least 500 in which the ethylene oxide and 1,2-propylene oxide are combined therein as oxy-

ethylene and oxy-1,2-propylene groups in a ratio from about one-third to one part 1,2-propylene oxide for each part of ethylene oxide by weight, the monoethers of said mixture containing in a single molecule both the oxyethylene and oxy-1,2-propylene groups and 30-60% by weight of glycerol monoricinoleate.

3. A gasoline-resistant grease comprising a gelling amount of a hydroxyalkylamine soap of an unsaturated fatty acid, 30-50% by weight of a mixture of monohydroxy oxyethylene oxy-1,2-propylene butyl monoethers having an average molecular weight of at least 900 in which ethylene oxide and 1,2-propylene oxide are combined therein as oxyethylene and oxy-1,2-propylene groups in a ratio from one part to nine parts of 1,2-propylene oxide for each part of ethylene oxide, by weight, the monoethers of said mixture containing in a single molecule both the oxyethylene and the oxy-1,2-propylene group, and 30-60% by weight of a partial ester of glycerine and a fatty acid having at least twelve carbon atoms.

4. A gasoline-resistant grease comprising a gelling proportion of a hydroxyalkylamine soap of an unsaturated hydroxy fatty acid, 30-50% by weight of a mixture of monohydroxy oxyethylene oxy-1,2-propylene butyl monoethers having an average molecular weight of at least 900 in which ethylene oxide and 1,2-propylene oxide are combined therein as oxyethylene and oxy-1,2-propylene groups in a ratio from one part to nine parts of 1,2-propylene oxide for each part of ethylene oxide, by weight, the monoethers of said mixture containing in a single molecule both the oxyethylene and the oxy-1,2-propylene group, and 30-60% by weight of a partial ester of glycerine and an unsaturated fatty acid having at least twelve carbon atoms.

5. A gasoline-resistant grease comprising a gelling amount of a hydroxyalkylamine soap of an unsaturated hydroxy fatty acid having at least twelve carbon atoms, 20-50% by weight of a mixture of monohydroxy oxyethylene oxy-1,2-propylene butyl monoethers having an average molecular weight of at least 900 in which ethylene oxide and 1,2-propylene oxide are combined therein as oxyethylene and oxy-1,2-propylene groups in a ratio from one part to nine parts of 1,2-propylene oxide for each part of ethylene oxide, by weight, the monoethers of said mixture containing in a single molecule both the oxyethylene and the oxy-1,2-propylene group, and 30-60% by weight of a partial ester of glycerine and an unsaturated fatty acid having at least twelve carbon atoms.

6. A gasoline-resistant grease comprising a gelling amount of triethanolamine soap of an unsaturated hydroxy fatty acid having at least twelve carbon atoms, 30-50% by weight of a mixture of monohydroxy oxyethylene oxy-1,2-propylene butyl monoethers having an average molecular weight of at least 900 in which ethylene oxide and 1,2-propylene oxide are combined therein as oxyethylene and oxy-1,2-propylene groups in a ratio from one part to nine parts of 1,2-propylene oxide for each part of ethylene oxide, by weight, the monoethers of said mixture containing in a single molecule both the oxyethylene and the oxy-1,2-propylene group, and 30-60% by weight of a partial ester of an unsaturated hydroxy fatty acid and a polyhydric alcohol having less than four carbon atoms.

7. A gasoline-resistant grease comprising a gelling amount of an alkanolamine soap of an

unsaturated hydroxy fatty acid having at least twelve carbon atoms, 30-50% by weight of a water soluble polyoxyalkylene fluid and 30-60% by weight of glyceryl monoricinoleate.

8. A gasoline-resistant grease comprising a 5 gelling amount of triethanolamine ricinoleate, 30-50% by weight of a water soluble polyoxyalkylene fluid and 30-60% by weight of a partial ester of an unsaturated higher hydroxy fatty acid and of a polyhydric alcohol having less than 10 four carbon atoms.

9. A gasoline-resistant grease comprising a gelling amount of an alkanolamine soap of an unsaturated hydroxy fatty acid having at least twelve carbon atoms, 30-50% by weight of a 15 water soluble polyoxyalkylene fluid, and 30-60% by weight of a glyceryl monoester of a fatty acid having at least twelve carbon atoms per molecule.

10. A gasoline-resistant grease comprising a gelling amount of trialkanolamine ricinoleate, 20 30-60% by weight of glyceryl monoricinoleate and 20-50% by weight of a mixture of mono-hydroxy oxyethylene oxy-1,2-propylene butyl monoethers having an average molecular weight of at least 900 in which ethylene oxide and 1,2- 25 propylene oxide are combined therein as oxyethylene and oxy-1,2-propylene groups in a ratio from one part to nine parts of 1,2-propylene oxide for each part of ethylene oxide, by weight, the monoethers of said mixture containing in 30 a single molecule both the oxyethylene and the oxy-1,2-propylene group, said composition also containing minor amounts sufficient to improve the oxidation and corrosion characteristics

thereof of phenyl-alpha-naphthylamine and of an oleic acid salt of 2-heptyl-4-hydroxymethyl-4-ethyloxazoline.

11. A gasoline-resistant grease comprising a gelling amount of a hydroxy alkylamine soap of a high fatty acid, 20-50% by weight of a water-soluble polyoxyalkylene fluid, 30-60% by weight of a partial ester of a polyhydric alcohol having less than 6 carbon atoms per molecule with a higher fatty acid, and minor amounts sufficient in combination to substantially improve the oxidation and corrosion stability of said composition of an aromatic amine and of a higher fatty acid salt of a substituted oxazoline having the general configuration:



wherein  $\text{R}_1$  and  $\text{R}_2$  are substituents of the group consisting of hydrogen, and alkyl, hydroxyalkyl, aryl and acyl-oxyalkyl radicals and  $\text{R}_3$  and  $\text{R}_4$  are radicals of the group consisting of hydrogen, and alkyl substituents.

HAROLD A. WOODS.  
LOREN C. BOLLINGER.

References Cited in the file of this patent  
UNITED STATES PATENTS

| Number    | Name                   | Date          |
|-----------|------------------------|---------------|
| 2,083,132 | Williams et al. -----  | June 8, 1937  |
| 2,425,845 | Toussaint et al. ----- | Aug. 19, 1947 |